

## UNITED STATES PATENT OFFICE

2,214,432

ALUMINUM ALLOY CONTAINING COPPER,  
IRON, AND COLUMBIUM

Alfred John Murphy, Petts Wood, and Stanley  
Alfred Edward Wells, Teddington, England, as-  
signors, by mesne assignments, to Electro Met-  
allurgical Company, New York, N. Y., a corpora-  
tion of West Virginia

No Drawing. Original application April 16, 1937,  
Serial No. 137,280. Divided and this applica-  
tion August 14, 1939, Serial No. 290,074. In  
Great Britain May 5, 1936

## 3 Claims. (Cl. 75—139)

This invention comprises improvements in alu-  
minum base alloys and in particular aluminum  
alloys of the classes containing copper, or nickel,  
or copper together with nickel, or copper with  
5 nickel and magnesium, or copper with nickel,  
magnesium, iron and silicon, or nickel with mag-  
nesium, iron and silicon. This application is a  
division of our application Serial No. 137,280, filed  
April 16, 1937.

10 In the production of cast pieces of aluminum  
base alloys, by which may be understood alloys  
containing more than 70% of aluminum, it is de-  
sirable to secure the finest possible size of grain.  
The grain referred to is the macrostructure,  
15 which is recognizable by the naked eye on smooth  
surfaces or sections of the cast pieces after they  
have been etched in suitable reagents, such as an  
aqueous solution of caustic soda, or hydrofluoric  
acid.

20 In castings a diminution in grain size im-  
proves the mechanical properties. The finer the  
grain size characteristic of an aluminum alloy,  
other things being equal, the better its founding  
25 properties in that the tendency to cracking in  
the mold is reduced and the production of sound  
castings is facilitated. In cast pieces intended  
to be forged, pressed, extruded or otherwise  
worked mechanically, a fine grain size is desir-  
30 able because it assists the attainment of good  
mechanical properties in the subsequent work-  
ing.

The object of the invention is to produce alu-  
minum alloys having a fine grain, and possessing  
in consequence of this fine grain superior  
35 mechanical properties in the cast condition and  
also when forged and also after heat-treatment  
of the castings and forgings according to known  
processes.

According to this invention, a relatively small  
40 proportion of columbium, also known sometimes  
as niobium, is added to an aluminum alloy,  
particularly an alloy of one of the classes  
referred to, the alloy thereby acquiring a fine  
grain, which is maintained over a wide range  
45 of conditions of melting, casting and working.  
We have found it convenient to make the pro-  
portion of columbium 0.1% to 0.2% of the total  
weight of the alloy. We have observed ap-  
preciable grain refinement with as little as 0.05%  
50 of columbium, and on the other hand we have  
not found it generally necessary or desirable to  
exceed 0.5% of columbium.

We have discovered that these beneficial  
effects are exhibited in the classes of alloy men-  
tioned above containing the elements set out

below in the proportions stated by way of  
example:

|           | Per cent   |
|-----------|------------|
| Copper    | 0.5 to 12  |
| Nickel    | 0.5 to 5   |
| Magnesium | 0.1 to 3   |
| Silicon   | 0.2 to 2.5 |
| Iron      | 0.2 to 2   |
| Columbium | 0.05 to 1  |

The beneficial effect of the columbium is not  
dependent upon the manner in which it is in-  
corporated in the alloy, but a convenient pro-  
cedure is to add it in the form of a "hardener"  
or "mother" alloy or prealloy relatively rich in  
columbium. According to one practical process,  
the first stage in the incorporation of the  
columbium in the aluminum alloy is the prepara-  
tion of an aluminum alloy relatively rich in  
columbium from ferro-columbium and alu-  
minum. The ferro-columbium may be in the  
form of an alloy containing approximately equal  
parts of iron and columbium with impurities  
such as tantalum, silicon and carbon in small  
proportions. In preparing the columbium  
"hardener" alloy, aluminum is melted in a  
crucible and its temperature raised to 1100° to  
1200° C. A weight of ferro-columbium equal to  
approximately one-tenth of the weight of alu-  
minum is stirred into the molten aluminum, or  
is carried in a perforated container which is 20  
moved up and down in the aluminum, until the  
addition is entirely dissolved. In this way an  
alloy containing approximately 5% columbium,  
5% iron, with the balance substantially alu-  
minum, is obtained. This is cast into molds, re-  
melted in a crucible, allowed to solidify and re-  
melted without unnecessary superheating, in  
order to eliminate gases which may have become  
absorbed through the heating to high tempera-  
tures in the initial operation. After this "pre- 40  
solidification" treatment, the alloy is cast into  
suitable ingot molds.

One practical process for making up an alloy  
using the aluminum "hardener" alloy relatively  
rich in columbium may be described. The final  
alloy to be made according to this example has  
the following nominal composition:

|           | Per cent  |
|-----------|-----------|
| Copper    | 2.5       |
| Nickel    | 1.5       |
| Magnesium | 0.8       |
| Silicon   | 1.2       |
| Iron      | 1.2       |
| Columbium | 0.1       |
| Aluminum  | Remainder |

The "hardener" alloys employed are: aluminum-nickel with 20% nickel, aluminum-iron-columbium with 5% iron and 5% columbium, aluminum-iron with 10% iron, aluminum-copper with 50% copper, aluminum-silicon with 20% silicon. Aluminum is melted in a crucible and the calculated quantities of "hardeners" are stirred in successively in the order in which they are mentioned above, care being taken that each 5 addition is dissolved before the next is introduced. The final addition is the magnesium in the form of the pure metal. By this procedure it is not necessary to raise the temperature of the metal above 750° C. at any stage during the 10 manufacture of the alloy, which is advantageous from the point of view of avoiding absorption of gas.

The alloy described is suitable for the manufacture of castings and forgings, and responds 20 effectively to the known processes of heat-treatment applicable to aluminum alloys containing copper, nickel, magnesium, silicon and iron. For example, a large improvement in mechanical 25 properties of forgings of the alloy is obtained by a two-stage heat-treatment in which the parts are first heated for 4 hours at 530° C., then quenched in water, reheated for 16 hours at 165° C. and finally quenched in water again.

A valuable feature of the grain refining action 30 of columbium is that it is effective even when the aluminum alloy is raised to a high temperature before casting. As an illustration of the

efficacy of the grain refining action of columbium, it may be mentioned that, when an alloy of the composition stated above is cast at 800° C. into a dried sand mold to form a cylindrical block 3" high and 3" diameter, the grains visible in 5 the macrostructure after etching have diameters of 0.2 to 1 mm., whereas the same alloy not containing columbium, cast under the same conditions, shows a grain diameter of 2.5 to 5 mm.

As compared with a similar alloy not containing 10 columbium, the alloy described above has the advantage, due to the fine grain structure which columbium confers, that the ductility associated with a certain tensile strength is greater.

In the simple alloys of aluminum with copper, 15 such as that containing 7% copper, the incorporation of columbium in the form of an aluminum-columbium alloy refines the grain and improves the strength and ductility of castings.

We claim:

1. Aluminum base alloy containing 0.5% to 12% copper, iron in a proportion not over 2%, 0.05% to 1% columbium, remainder aluminum.
2. Aluminum base alloy containing 0.5% to 12% copper, iron in a proportion not over 2%, 25 0.1% to 0.5% columbium, remainder aluminum.
3. Alloy as defined in claim 2, wherein the proportion of copper is about 7% and the proportion of columbium is 0.1% to 0.2%.

ALFRED JOHN MURPHY.

STANLEY ALFRED EDWARD WELLS.

30